# EUROPEAN PATENT SPECIFICATION

(11) **EP 0 695 812 B1**
(45) Date of publication and mention of the grant of the patent: **12.01.2000**
(21) Application number: 95111776.1
(22) Date of filing: 26.07.1995
(51) Int. Cl.: C22C 45/02, H01F 1/153, H01F 3/04

(54) **Nanocrystalline alloy with insulating coating, magnetic core made thereof, and process for forming insulating coating on a nanocrystalline alloy**
Nanokristalline Legierung mit isolierender Beschichtung, daraus hergestellter Magnetkern und Verfahren zur Herstellung einer isolierenden Beschichtung auf der nanokristallinen Legierung
Alliage nanocristallin muni d'un revêtement isolant, noyau magnétique fabriqué avec cet alliage et procédé pour former un revêtement isolant sur cet alliage nanocristallin

(30) Priority: 01.08.1994 JP 18003794
(43) Date of publication of application: 07.02.1996
(73) Proprietor: HITACHI METALS, LTD., Chiyoda-ku, Tokyo (JP)
(72) Inventor: Yoshizawa, Yoshihito, Fukaya-shi, Saitama-ken (JP)
(74) Representative: Strehl Schübel-Hopf & Partner

(56) References cited:
- EP-A- 0 400 550
- EP-A- 0 585 940
- US-A- 5 083 366

## Description

### BACKGROUND OF THE INVENTION

The present invention relates to nanocrystalline alloy having an insulating coating thereon, which is excellent in high-frequency characteristics and suitable for use in various magnetic parts such as transformer, choke coil, etc., and further relates to a magnetic core made of the nanocrystalline alloy and a method for forming the insulating coating on the nanocrystalline alloy.

A nanocrystalline alloy, which contains fine crystal grains having an average grain size of 50 nm or less in an area ratio of 50% or more of the alloy structure, has been, because of its good soft magnetic properties, used for producing magnetic cores of a common-mode choke coil, a high-frequency transformer, an electrical leak alarm, pulse transformer, etc. Typical examples for such a nanocrystalline alloy are disclosed in U.S. Patent No. 4,881,989 and JP-A-1-242755. The nanocrystalline alloy known in the art has been generally produced by subjecting an amorphous alloy obtained by quenching a molten or vaporized alloy to a heat treatment for forming fine crystals. A method for quenching a molten alloy to produce an amorphous alloy may include a single roll method, a twin roll method, a centrifugal quenching method, a rotation spinning method, an atomization method, a cavitation method, etc. A method for quenching a vaporized metal may include a sputtering method, a vapor deposition method, an ion plating method, etc. The nanocrystalline alloy is produced by finely crystallizing an amorphous alloy produced by the above method, and is known to have, contrary to amorphous alloys, a good heat stability as well as a high saturation magnetic flux density, a low magnetostriction, and a good soft magnetic property. The nanocrystalline alloy is also known to show a little change with time in its properties and have a good temperature stability.

Conventionally, the magnetic core used in a noise filter, a pulse transformer, etc. has been made of a highly permeable material having good high-frequency characteristics such as ferrite, an amorphous alloy, etc. In a high-frequency transformer for an inverter, a material low in the magnetic core loss has been used. Further, the Fe-based nanocrystalline alloy disclosed in U.S. Patent No. 4,881,989 is described to have a high permeability and a low magnetic core loss, and therefore, suitable for the use mentioned above.

However, it has been found by the inventor that a magnetic core for a common-mode choke coil or a high-frequency magnetic core for an inverter transformer made of thin ribbon of an Fe-based nanocrystalline alloy does not exhibit sufficient properties when the surface of the thin ribbon is not smooth and the thin ribbons are not subjected to layer insulation because the influence of eddy current on the properties comes to remarkable with increasing width of the thin ribbon. As a method of layer insulation, JP-A-63-302504 and US-A-5 083 366 discloses to apply SiO₂ powder or MgO powder on a part of or complete surface of a thin alloy ribbon or to coat a thin alloy ribbon with an alcohol solution of a modified alkyl silicate added with an acid. JP-A-2-297903 discloses to form a heat-resistant insulating layer of 0.5-5 µm thick by heating a coating comprising a uniform mixture of 20-90 weight % (calculated in terms of SiO₂) of a silanol oligomer and 80-10 weight % of a ceramic fine particle to allow the oligomers cross-linked each other.

However, since an amorphous alloy contracts during the heat treatment for nanocrystallization, an insulating layer on the alloy is cracked or separated from the surface of the alloy due to the contraction stress. Also, sufficient magnetic properties cannot be attained due to the internal stress of the alloy generated by contraction. Although the method disclosed in JP-A-2-297903 solved these problems, the insulating layer formed by the method has a poor affinity for a resin. Therefore, when a magnetic core, for example, for an inverter transformer made of a thin alloy ribbon having such an insulating layer is cut after impregnation with a resin, the resin exfoliates from the cut surface and the thin alloy ribbons are not laminated each other. In the method wherein SiO₂ powder or MgO powder is applied on the surface of an alloy, the powder is likely to be separated from the alloy surface during the production of the magnetic core to lead to insufficient insulation.

The influence of the contraction by the heat treatment is not necessary to be considered when an amorphous alloy provided with an insulating coating is produced. However, as described above, the contraction during the heat treatment causes defective insulation due to cracking or peeling of the insulating coating or deterioration of magnetic properties due to increased internal stress. Therefore, an insulating coating free from the above problems and a method for forming such an insulating coating on a nanocrystalline alloy has been demanded to be developed. Further, an insulating coating exhibiting sufficient insulation properties even if the insulating coating is made thinner has been required in the field of electronic circuitry which requires a small-sized magnetic core.

Accordingly, an object of the present invention is to provide a nanocrystalline alloy excellent in insulating properties. Another object of the present invention is to provide a magnetic core excellent in magnetic properties at high frequency, and still another object of the present invention is to provide a method for forming an insulating coating free from the conventional problems.

As a result of the intense research in view of the above objects, the inventor have found that an insulating coating formed by heating a solution of at least one insulating material selected from the group consisting of aluminum silicates, lithium silicates and magnesium methylate is free from cracking and peeling during the heat treatment for crystallization of an amorphous alloy, and a nanocrystalline alloy provided with such an insulating coating is excellent in insulating properties and suitable as a material for magnetic core used at high frequency. The present invention has been accomplished based on the finding.

Thus, in a fist aspect of the present invention, there is provided a nanocrystalline alloy having on at least one surface thereof an insulating coating, the nanocrystalline alloy having a chemical composition represented by the following formula:

(Fe₁₋ₐMₐ)_{100-x-y-z-b}AₓM'_{y}M"_{z}X_{b} (by atomic %),

wherein M is at least one element selected from the group consisting of Co and Ni, A is at least one element selected from the group consisting of Cu and Au, M' is at least one element selected from the group consisting of Ti, V, Zr, Nb, Mo, Hf, Ta and W, M" is at least one element selected from the group consisting of Cr, Mn, Al, Sn, Zn, Ag, In, platinum group elements, Mg, Ca, Sr, Y, rare earth elements, N, O and S, X is at least one element selected from the group consisting of B, Si, C, Ge, Ga and P, and each of a, x, y, z and b respectively satisfies 0≤ a≤ 0.5, 0≤ x≤ 10, 0. 1≤ y≤ 20, 0≤ z≤ 20 and 2≤ b≤ 30, and the insulating coating having an average thickness of 2 µm or less and consisting of at least one insulating material selected from the group consisting of aluminum silicates, lithium silicate and magnesium oxide.

In a second aspect of the present invention, there is provided a magnetic core made of the nanocrystalline alloy as defined above.

In a third aspect of the present invention, there is provided a method for forming an insulating coating on a nanocrystalline alloy, which comprises (1) rapidly quenching a molten alloy having a chemical composition represented by the following formula:

(Fe₁₋ₐMₐ)_{100-x-y-z-b}AₓM'_{y}M''_{z}X_{b} (by atomic %),

wherein M is at least one element selected from the group consisting of Co and Ni, A is at least one element selected from the group consisting of Cu and Au, M' is at least one element selected from the group consisting of Ti, V, Zr, Nb, Mo, Hf, Ta and W, M'' is at least one element selected from the group consisting of Cr, Mn, Al, Sn, Zn, Ag, In, platinum group elements, Mg, Ca, Sr, Y, rare earth elements, N, O and S, X is at least one element selected from the group consisting of B, Si, C, Ge, Ga and P, a, x, y, z and b satisfy 0≤ a≤ 0.5, 0≤ x≤ 10, 0. 1≤ y≤ 20, 0≤ z≤ 20 and 2≤ b≤ 30, to produce an amorphous alloy; (2) coating on at least one surface of the amorphous alloy a solution containing at least one insulating material selected from the group consisting of aluminum silicates, lithium silicate and magnesium methylate; (3) drying the solution-coated amorphous alloy at a temperature between 80°C and 350°C; and (4) heat-treating the dried amorphous alloy at a temperature not lower than a crystallization temperature of said amorphous alloy so as to form a fine crystal grain having a grain size of 30 nm or less in alloy structure while forming said insulating coating having a thickness of 2 µm or less and consisting of at least one insulating material selected from the group consisting of aluminum silicates, lithium silicate and magnesium oxide.

### BRIEF DESCRIPTION OF THE DRAWINGS

Fig. 1 is a schematic representation illustrative of one embodiment of the method of the present invention;
Fig. 2 is a schematic representation illustrative of another embodiment of the method of the present invention;
Fig. 3 is a schematic representation illustrative of still another embodiment of the method of the present invention; and
Fig. 4 is a schematic view showing a toroidal magnetic core of the present invention.

### DETAILED DESCRIPTION OF THE INVENTION

The nanocrystalline alloy of the present invention which has an insulating coating on at least one surface thereof may be produce as described below.

First, an amorphous alloy is produced by rapidly quenching a molten alloy having a chemical composition represented by the following formula:

(Fe₁₋ₐMₐ)_{100-x-y-z-b}AₓM'_{y}M''_{z}X_{b} (by atomic %),

wherein M is at least one element selected from the group consisting of Co and Ni, A is at least one element selected from the group consisting of Cu and Au, M' is at least one element selected from the group consisting of Ti, V, Zr, Nb, Mo, Hf, Ta and W, M'' is at least one element selected from the group consisting of Cr, Mn, Al, Sn, Zn, Ag, In, platinum group elements, Mg, Ca, Sr, Y, rare earth elements, N, O and S, X is at least one element selected from the group consisting of B, Si, C, Ge, Ga and P, a, x, y, z and b satisfy 0≤ a≤ 0.5, 0≤ x≤ 10, 0. 1≤ y≤ 20, 0≤ z≤ 20 and 2≤ b≤ 30. A single-roll method, a twin-roll method, etc. may be employed to rapidly quenching the molten alloy.

A chemical composition out side the above range fails to give a sufficient effect attained by the present invention due to a remarkable reduction in specific permeability or a remarkable increasing in magnetic core lose, thereby making it unable to obtain a nanocrystalline alloy of practical characteristics.

Then, a solution of at least one insulating material is applied on at least one surface of the amorphous alloy thus produced. The insulating material is selected from the group consisting of aluminum silicates, modified aluminum silicates, lithium silicates and magnesium methylate. The concentration of the insulating material in the solution is preferably 5 to 50 % by weight. The solution thus prepared may be mixed with a solution of colloidal silica. The solution may be applied on an amorphous alloy after subjecting the amorphous alloy to anodizing treatment which improves the insulating properties and corrosion resistance of the resulting nanocrystalline alloy. The amount of the solution being applied on the amorphous alloy is regulated so that the thickness of the resulting insulating coating may be 2 µm or less.

The amorphous alloy applied with the solution is then dried at a temperature of 80-350°C, preferably for 5 seconds to 10 minutes. The drying may be effected by blowing the applied solution with air or another gas such as argon, nitrogen, helium, etc. maintained at 80-350°C to rapidly dry the solution. This makes the insulating coating uniform in its thickness.

Before subjected to the subsequent heat treatment, the amorphous alloy thus dried is usually made into a form of magnetic core by winding the thin ribbon of amorphous alloy or laminating cut sheets or punched sheets of the amorphous alloy. The winding or laminating step may be carried out after heat treatment when the heat-treated alloy ribbon is sufficiently flexible.

The heat treatment for crystallization is carried out at a temperature not lower than the crystallization temperature of the amorphous alloy, usually at 450-700°C, for 1 minute to 24 hours in an inert gas atmosphere such as nitrogen gas atmosphere, argon gas atmosphere, etc. or an oxidizing atmosphere such as air. By this heat treatment, fine crystal grains are formed in the alloy structure, and simultaneously, the insulating coating is formed on the surface of the resulting nanocrystalline alloy. During the heat treatment, the magnesium methylate is oxidized to provide an insulating coating comprising magnesium oxide.

When an amorphous alloy applied with the solution is directly subjected to heat treatment without being dried, the heat-treatment atmosphere comes to contain a large amount of moisture evaporated form the solution. This leads to a preferential crystallization of the surface of the alloy. As a result, a nanocrystalline alloy of a uniform and fine structure cannot be obtained. Also, cracking and peeling of the insulating coating are likely to occur. Therefore, the drying step prior to the heat treatment of crystallization is indispensable.

The production method of the present invention will be further described while referring to the drawings.

In Fig. 1, a thin ribbon 1 of amorphous alloy, which is unwound in the direction indicated by the arrow from a winding reel 2, is allowed to pass through a solution 4 stored in a vessel 3 to apply the solution 4 on both the surface of the thin ribbon 1 of amorphous alloy. After passing through a scraper 5, the thin ribbon 1 of amorphous alloy is introduced into a drying furnace 6 kept at 80- 350°C. The dried thin ribbon 1 of amorphous alloy is then wound on a winding reel 7 and subjected to the subsequent heat treatment of crystallization.

In Fig. 2, a thin ribbon 1 of amorphous alloy, which is unwound in the direction indicated by the arrow from a winding reel 2, is allowed to pass through a roll coater 8. A transfer roll 10 is partially immersed in a solution 4 stored in a vessel 3 to apply the solution 4 on the lower surface of the thin ribbon 1 of amorphous alloy, which is then introduced into a drying furnace 6 kept at 80 - 350°C. The dried thin ribbon 1 of amorphous alloy is then wound on a winding reel 7 and subjected to the subsequent heat treatment of crystallization.

In Fig. 3, the upper surface of a thin ribbon 1 of amorphous alloy, which is unwound in the direction indicated by the arrow from a winding reel 2, is sprayed with a solution 4 from a spray 9. The thin ribbon 1 of amorphous alloy is then introduced into a drying furnace 6 kept at 80-350°C. The dried thin ribbon 1 of amorphous alloy is then wound on a winding reel 7 and subjected to the subsequent heat treatment of crystallization.

The nanocrystalline alloy produced by the method described above has preferably a thickness of 2 to 50 µm and contains fine crystals having an average grain size of 30 nm or less, preferably in an area ratio of 50 % or more. The fine crystals mainly comprise bcc Fe-phase (body centered cubic lattice phase) containing Si, and may contain an ordered lattice phase or are constituted of ordered lattice. Alloying elements other than Si, i.e., B, Al, Ge, Zr, etc. may be contained as a solid solution component in the bcc Fe-phase. The remaining part other than the crystal phase mainly comprises amorphous phase. However, a nanocrystalline alloy substantially comprising only crystal phase is also embraced within the scope of the present invention. A compound phase may also be formed in a part of the alloy structure.

The average thickness of the insulating coating is 2 µm or less, preferably 0.01 to 1 µm. An average thickness of 0.5 µm or less is particularly preferred because the size of magnetic core can be reduced while maintaining its excellent insulating properties.

A solution of aluminum silicate (Al₂O₃•SiO₂) provides the surface of nanocrystalline alloy with an insulating coating having a uniform thickness and a high resistance to peeling because internal stress is hardly generated in the alloy during the crystallization process. Therefore, the insulating properties can be improved. A nanocrystalline alloy having such an insulating coating exhibits a high permeability and a low magnetic core loss at low and high frequency range.

A solution of lithium silicate (Li₂O•SiO₂) produces the same effect as above because internal stress is hardly generated in the alloy during the crystallization process.

Since a solution of magnesium methylate can be dried rapidly, a thin, uniform and hard insulating coating comprising magnesium oxide, which exhibits improved insulating properties, is formed on the nanocrystalline alloy.

The magnetic core made by laminating or winding the nanocrystalline alloy described above is excellent in layer insulation and has little internal stress, and therefore, suitable for magnetic core used in a high-frequency range. In addition, since the nanocrystalline alloy has a good affinity for a resin such as an epoxy-type resin, a cut core having a high interlaminar strength can be obtained.

The present invention will be further described while referring to the following Examples which should be considered to illustrate various preferred embodiments of the present invention.

### Example 1

An amorphous alloy ribbon having a width of 25.4 mm and a thickness of 18 µm was produced by quenching a molten alloy of F_{bal.}Cu_{0.9}Nb_{2.8}Si_{15.5}B_{6.2}(atomic %) by using a single roll method. After being passed through a solution containing each insulating material listed in Table 1, the amorphous alloy ribbon was dried in a hot-gas furnace kept at 200°C. The dried amorphous alloy ribbon was then wound to form a toroidal shape of 100 mm outer diameter and 80 mm inner diameter, and then heated to 570°C in a furnace at a heating rate of 1 .5°C/min and maintained there for 15 minutes to be subjected to heat treatment in a nitrogen atmosphere. The heat-treated product was cooled to room temperature to obtain each magnetic core. The most part of the alloy structure of the resulting nanocrystalline alloy was occupied with extremely fine grains comprising bcc-phase of an average grain size of about 12 nm.

For comparison, a toroidal magnetic core having no insulating coating was produced in the same manner as above (Sample No. 9).

The specific permeability (µᵣ) at 10 MHz, the magnetic core loss (Pc) at 500 kHz and 0.05 T, the average thickness of the insulating coating and the resistance (R) between the innermost part and the surface of the magnetic core are shown in Table 1.

**Table 1**

| Sample No | Insulating Material | | Pc | R | Thickness |
|---|---|---|---|---|---|
| | | µᵣ | (kW/m³) | (Ω) | (µm) |
| Invention | | | | | |
| 1 | modified aluminum silicate | 640 | 220 | 135 | 0.8 |
| 2 | lithium silicate | 650 | 220 | 138 | 0.7 |
| 3 | magnesium methylate | 590 | 240 | 128 | 0.2 |
| 4 | lithium silicate | 710 | 210 | 142 | 1.2 |
| 5 | magnesium methylate | 620 | 260 | 121 | 0.1 |

| Comparison | | | | | |
|---|---|---|---|---|---|
| 6 | alumina sol | 410 | 360 | 27 | 1.1 |
| 7 | alkyl silicate | 490 | 310 | 35 | 1.2 |
| 8 | colloidal silica | 480 | 330 | 29 | 0.2 |
| 9 | - | 120 | 590 | 1.1 | - |

As seen from Table 1, the nanocrystalline alloy having the insulating coating of the present invention had a large value of R, which means a high interlaminar insulating resistance. This results in high magnetic properties of a high µᵣ and a low Pc.

### Example 2

An amorphous alloy ribbon having a width of 20 mm and a thickness of 18 µm was produced by quenching a molten alloy having each chemical composition shown in Table 2 by using a single roll method. After being passed through a solution dissolving each insulating material listed in Table 2, the amorphous alloy ribbon was dried in a hot-gas furnace kept at 200°C. The dried amorphous alloy ribbon was then wound to form a toroidal shape of 100 mm outer diameter and 80 mm inner diameter, and then heated to 570°C in a furnace at a heating rate of 1 . 5°C/min and maintained there for 15 minutes to be subjected to heat treatment in a nitrogen atmosphere. The heat-treated product was cooled to room temperature to obtain each magnetic core. The most part of the alloy structure of the resulting nanocrystalline alloy was occupied with extremely fine grains comprising bcc-phase of an average grain size of about 12 nm.

The specific permeability (µᵣ) at 10 MHz, the magnetic core loss (Pc) at 500 kHz and 0.05 T, the average thickness of the insulating coating and the resistance (R) between the innermost part the surface of the magnetic core are shown in Table 2.

**Table 2**

| Sample No. | Composition (atomic %) | Insulating Material | | |
|---|---|---|---|---|
| Invention | | | | |
| 10 | Fe_{bal.}Cu₁Hf₂Si₉B₁₃ | modified aluminum silicate | | |
| 11 | Fe_{bal.}Cu₁Nb₇B₉Ge₄ | lithium silicate | | |
| 12 | Fe_{bal.}Cu₁Nb₃Y₁Si_{16.5}B₆ | magnesium methylate | | |
| 13 | Fe_{bal}.Cu_{1.6}Nb₂W₁Si₁₆B₆P₁ | lithium silicate | | |
| 14 | Fe_{bal}.Au₁Nb₂Mn₁Si₁₃B₇ | magnesium methylate | | |
| 15 | Fe_{bal.}Cu₁Nb₃Si₁₅B₇Ga_{0.001} | lithium silicate | | |
| 16 | Fe_{bal}.Cu₁MO₅Si₁₆B₇C₁ | magnesium methylate | | |
| 17 | Fe_{bal}.Au₁Ti₁Nb₂Si₁₄B₇S_{0.001} | lithium silicate | | |
| 18 | Fe_{bal.}Cu₁Nb_{2.5}Si₁₄B₆Al₂ | modified aluminum silicate | | |
| 19 | Fe_{bal.}Ni₁Cu₁Nb₃Si₁₅B₇N_{0.001} | magnesium methylate | | |
| 20 | Fe_{bal.}Co₁Cu₁Nb₃Si₁₅B₇Sn_{0.06} | lithium silicate | | |
| 21 | Fe_{bal.}Cu₁Nb₃Ru₁Si₁₅B₆In_{0.06} | modified aluminum silicate | | |
| 22 | Fe_{bal.}Au₁Nb₂Pd₁Si₁₈B₇S_{0.001} | magnesium methylate | | |

| Comparison | | | | |
|---|---|---|---|---|
| 23 | Fe_{bal}.Cr₁Si₉B₁₃ (amorphous) | alumina sol | | |
| 24 | Fe_{bal.}Cr₁Si₉B₁₃) | (amorphous) magnesium methylate | | |

| Sample No. | µᵣ | Pc (kW/m³) | R (Ω) | Thickness (µm) |
|---|---|---|---|---|
| Invention | | | | |
| 10 | 610 | 240 | 143 | 2 |
| 11 | 510 | 290 | 121 | 0.2 |
| 12 | 590 | 300 | 114 | 0.1 |
| 13 | 580 | 260 | 101 | 0.1 |
| 14 | 570 | 270 | 98 | 0.05 |
| 15 | 580 | 260 | 99 | 0.09 |
| 16 | 590 | 250 | 111 | 0.12 |
| 17 | 600 | 220 | 100 | 0.1 |
| 18 | 510 | 390 | 112 | 0.15 |
| 19 | 610 | 210 | 114 | 0.14 |
| 20 | 610 | 210 | 108 | 0.15 |
| 21 | 520 | 370 | 105 | 0.14 |
| 22 | 610 | 210 | 111 | 0.12 |

| Comparison | | | | |
|---|---|---|---|---|
| 23 | 140 | 650 | 105 | 0.12 |
| 24 | 170 | 600 | 111 | 0.12 |

From Table 2, the magnetic core of the present invention is found to be excellent because of its high permeability (µᵣ) and low magnetic core loss (Pc).

### Example 3

An amorphous alloy ribbon having a width of 20 mm and a thickness of 12 µm was produced by quenching a molten alloy of Fe_{bal.}Cu₁Nb₃Si₁₆B_{6.5}Cr_{0.5}Sn_{0.05} (atomic %) by using a single roll method. After being passed through a solution of lithium silicate, the amorphous alloy ribbon was dried in a hot-gas furnace kept at each temperature listed in Table 3. The dried amorphous alloy ribbon having a coating of about 1 µm thick was then wound to form a toroidal shape of 60 m m outer diameter and 50 mm inner diameter, and then heated to 570°Cin a furnace at a heating rate of 1.2°C/min and maintained there for 15 minutes to be subjected to heat treatment in a nitrogen atmosphere. The heat-treated product was cooled to room temperature to obtain each magnetic core. The most part of the alloy structure of the resulting nanocrystalline alloy was occupied with extremely fine grains comprising bcc-phase of an average grain size of about 12 nm.

The specific permeability (µᵣ) at 1 kHz of each magnetic core is shown in Table 3.

Further, the brittleness of each nanocrystalline alloy was evaluated bywhether brittle fracture occurred when the alloy was bent.

**Table 3**

| Sample No. | Drying Temperature (°C) | µᵣ | Brittle Fracture |
|---|---|---|---|
| Invention | | | |
| 25 | 80 | 91200 | None |
| 26 | 100 | 93200 | None |
| 27 | 150 | 94500 | None |
| 28 | 200 | 96800 | None |
| 29 | 250 | 96700 | None |
| 30 | 300 | 95800 | None |
| 31 | 350 | 96100 | None |

| Comparison | | | |
|---|---|---|---|
| 32 | 40 | 73200 | None |
| 33 | 60 | 85900 | None |
| 34 | 380 | - | Observed |
| 35 | 400 | - | Observed |

When the drying temperature was lower than 80°C (Sample Nos. 32 and 33), the alloy ribbons after heat treatment for crystallization were stuck each other because of insufficient drying to result in reduced magnetic properties. On the other hand, when the dried temperature was higher than 350°C (Sample Nos. 34 and 35), the alloy ribbons were embrittled and easily broken. This made the production of the magnetic core very difficult, and therefore, the permeability (µᵣ) was unable to be determined.

### Example 4

An amorphous alloy ribbon having a width of 25 mm and a thickness of 12 µm was produced by quenching a molten alloy of Fe_{bal.}Nb₃Ga₄Si₁₄B₇ (atomic %) by using a single roll method. After being passed through a solution containing each insulating material listed in Table 4, the amorphous alloy ribbon was dried in a hot-gas furnace kept at 200°C. The dried amorphous alloy ribbon was then wound to form a toroidal shape shown in Fig. 4, and then heated to 550°C in a furnace at a heating rate of 1. 2°C/min and maintained there for 15 minutes to be subjected to heat treatment in a nitrogen atmosphere. The heat-treated product was cooled to room temperature to obtain each magnetic core. The most part of the alloy structure of the resulting nanocrystalline alloy was occupied with extremely fine grains comprising bcc-phase of an average grain size of about 14 nm. Each magnetic core was impregnated with an epoxy-type resin and made into a cut core by cutting after the impregnated resin was hardened. The average thickness of the insulating coating, the magnetic core loss (Pc) at 20 kHz and 0.2 T, the resistance (R) between the innermost part and the surface and the appearance of the cut surface of each magnetic core are shown in Table 4.

**Table 4**

| Sample No. | Insulating Material | Thickness (µm) | Pc (kW/m³) | R (Ω) | Appearance of cut surface |
|---|---|---|---|---|---|
| Invention | | | | | |
| 36 | aluminum silicate | 0.8 | 42 | 83 | + |
| 37 | lithium silicate | 0.2 | 38 | 95 | + |
| 38 | magnesium methylate | 0.05 | 42 | 81 | + |
| 39 | lithium silicate | 0. 1 | 41 | 80 | + |
| 40 | magnesium methylate | 0.1 | 41 | 88 | + |

| Comparison | | | | | |
|---|---|---|---|---|---|
| 41 | alumina sol | 1.2 | 68 | 32 | - |
| 42 | alkyl silicate | 1.8 | 62 | 41 | - |
| 43 | - | 0 | 120 | 0.9 | + |
| Note: "+" means that no exfoliation of the resin and no interlaminar separation were observed at the cut surface, while "-" means that such were observed. | | | | | |

As seen from Table 4, no exfoliation of the resin and no interlaminar separation were observed at the cut surface in the magnetic cores of the present invention, this resulting in a low magnetic core loss. Further, the higher values of R show that the magnetic cores of the present invention are provided with sufficient layer insulation.

### Example 5

An amorphous alloy ribbon having a width of 20 mm and a thickness of 15 µm was produced by quenching a molten alloy of Fe_{bal.}Cu₁Ta₃Si₁₆B₆ (atomic %) by using a single roll method. After coating on the surface of the amorphous alloy a solution of each insulating material listed in Table 5 by using a roll coater, the amorphous alloy ribbon was dried in a hot-gas furnace kept at 20 °C. The dried amorphous alloy ribbon was then wound to form a toroidal shape of 35 mm outer diameter and 30 mm inner diameter, and then heated to 550°C in a furnace at a heating rate of 1 . 5°C/min and maintained there for 15 minutes to be subjected to heat treatment in a nitrogen atmosphere. The heat-treated product was cooled to room temperature to obtain each magnetic core. The most part of the alloy structure of the resulting nanocrystalline alloy was occupied with extremely fine grains comprising bcc-phase of an average grain size of about 12 nm.

The specific permeability (µᵣ) at 10 MHz, the magnetic core loss (Pc) at 500 kHz and 0.05 T, the average thickness of the insulating coating and the resistance (R) between the innermost part and the surface of the magnetic core are shown in Table 5.

**Table 5**

| Sample No. | Insulating Material | µᵣ | Pc (kW/m ³ ) | R (Ω) | Thickness (µm) |
|---|---|---|---|---|---|
| Invention | | | | | |
| 44 | aluminum silicate | 640 | 230 | 28.0 | 0.2 |
| 45 | lithium silicate | 650 | 220 | 29.1 | 0.1 |
| 46 | magnesium methylate | 650 | 210 | 29.2 | 0.01 |
| 47 | lithium silicate | 610 | 240 | 27.6 | 0.05 |
| 48 | magnesium methylate | 630 | 220 | 28.7 | 0.05 |

| Comparison | | | | | |
|---|---|---|---|---|---|
| 49 | alumina sol | 380 | 350 | 6.2 | 0.8 |
| 50 | alkyl silicate | 460 | 320 | 7.1 | 1.1 |

As seen from Table 5, the magnetic cores of the present invention were superior to the comparative magnetic cores because of their high permeabilities, low magnetic core losses and high insulating resistances.

### Example 6

An amorphous alloy ribbon having a width of 25 mm and a thickness of 15 µm was produced by quenching a molten alloy of F_{bal.}Cu₁Zr₃Si_{14.5}B_{6.5} (atomic %) by using a single roll method. After spraying on the surface of the amorphous alloy a solution of each insulating material listed in Table 6, the amorphous alloy ribbon was dried in a hot-gas furnace kept at 200°C. The dried amorphous alloy ribbon was then wound to form a toroidal shape of 50 mm outer diameter and 30 mm inner diameter, and then heated to 550°C in a furnace at a heating rate of 1 . 5°C/min and maintained there for 15 minutes to be subjected to heat treatment in a nitrogen atmosphere. The heat-treated product was cooled to room temperature to obtain each magnetic core. The most part of the alloy structure of the resulting nanocrystalline alloy was occupied with extremely fine grains comprising bcc-phase of an average grain size of about 12 nm.

The specific permeability (µᵣ) at 10 MHz, the magnetic core loss (Pc) at 500 kHz and 0.05 T, the average thickness of the insulating coating and the resistance (R) between the innermost part and the surface of the magnetic core are shown in Table 6.

**Table 6**

| Sample No. | Insulating Material | µᵣ | Pc (kW/m³) | R (Ω) | Thickness (µm) |
|---|---|---|---|---|---|
| Invention | | | | | |
| 51 | aluminum silicate | 610 | 240 | 90.5 | 0.8 |
| 52 | lithium silicate | 650 | 220 | 91.3 | 0.3 |
| 53 | magnesium methylate | 640 | 230 | 89.5 | 0.1 |
| 54 | lithium silicate | 560 | 250 | 87.6 | 0.2 |
| 55 | magnesium methylate | 550 | 260 | 86.6 | 0.06 |

| Comparison | | | | | |
|---|---|---|---|---|---|
| 56 | alumina sol | 340 | 360 | 21.1 | 1.3 |
| 57 | alkyl silicate | 390 | 330 | 23.1 | 1.1 |

As seen from Table 6, the magnetic cores of the present invention were superior to the comparative magnetic cores because of their high permeabilities, low magnetic core losses and high insulating resistances.

## Claims

1. A nanocrystalline alloy having on at least one surface thereof an insulating coating, said nanocrystalline alloy having a chemical composition represented by the following formula:
(Fe₁₋ₐMₐ)_{100-x-y-z-b}AₓM'_{y}M''_{z}X_{b} (by atomic %),
wherein M is at least one element selected from the group consisting of Co and Ni, A is at least one element selected from the group consisting of Cu and Au, M' is at least one element selected from the group consisting of Ti, V, Zr, Nb, Mo, Hf, Ta and W, M'' is at least one element selected from the group consisting of Cr, Mn, Al, Sn, Zn, Ag, In, platinum group elements, Mg, Ca, Sr, Y, rare earth elements, N, O and S, X is at least one element selected from the group consisting of B, Si, C, Ge, Ga and P, a, x, y, z and b satisfy 0≤ a≤ 0.5, 0≤ x≤ 10, 0. 1≤ y≤ 20, 0≤ z≤ 20 and 2≤ b≤ 30, and said insulating coating having an average thickness of 2 µm or less and consisting of at least one insulating material selected from the group consisting of aluminum silicates, lithium silicate and magnesium oxide.

2. The nanocrystalline alloy according to claim 1, wherein the average thickness of said insulating coating is 0.2 µm or less.

3. A magnetic core produced by laminating or winding said nanocrystalline alloy according to claim 1 or 2.

4. The magnetic core according to claim 3, which is impregnated with an epoxy-type resin.

5. A method for forming an insulating coating on a nanocrystalline alloy, which comprises:
rapidly quenching a molten alloy having a chemical composition represented by the following formula:
(Fe₁₋ₐMₐ)_{100-x-y-z-b}AₓM'_{y}M"_{z}X_{b} (by atomic %),
wherein M is at least one element selected from the group consisting of Co and Ni, A is at least one element selected from the group consisting of Cu and Au, M' is at least one element selected from the group consisting of Ti, V, Zr, Nb, Mo, Hf, Ta and W, M" is at least one element selected from the group consisting of Cr, Mn, Al, Sn, Zn, Ag, In, platinum group elements, Mg, Ca, Sr, Y,rare earth elements, N,Oand S,Xis at least one element selected from the group consisting of B, Si, C, Ge, Ga and P, a, x, y, z and b satisfy 0≤ a≤ 0.5, 0≤ x≤ 10, 0.1≤ y≤ 20, 0≤ z≤ 20 and 2≤ b≤ 30, to produce an amorphous alloy;
coating on at least one surface of said amorphous alloy a solution containing at least one insulating material selected from the group consisting of aluminum silicates, lithium silicate and magnesium methylate;
drying the solution-coated amorphous alloy at a temperature between 80°C and 350°C; and
heat-treating the dried amorphous alloy at a temperature not lower than a crystallization temperature of said amorphous alloy so as to form a fine crystal grain having a grain size of 30 nm or less in alloy structure while forming said insulating coating having a thickness of 2 µm or less and consisting of at least one insulating material selected from the group consisting of aluminum silicates, lithium silicate and magnesium oxide.

6. The method according to claim 5, wherein said solution is coated on said amorphous alloy by passing said amorphous alloy though said solution.

7. The method according to claim 5, wherein said solution is coated on said amorphous alloy by passing said amorphous alloy though a roll coater.

8. The method according to claim 5, wherein said solution is coated on said amorphous alloy by spraying said solution on the surface of said amorphous alloy.

9. The method according to any one of claims 5 to 8, wherein said amorphous alloy is coated with said solution after the surface of said amorphous alloy is subjected to anodizing treatment.

10. The method according to any one of claims 5 to 9, wherein said amorphous alloy coated with said solution is dried by blowing a hot air, argon gas, nitrogen gas or helium gas onto the surface of said amorphous alloy.

## Revendications

1. Alliage nanocristallin ayant sur au moins une surface de celui-ci un revêtement isolant, ledit alliage nanocristallin ayant une composition chimique représentée par la formule suivante :
(Fe_{1 - a}Mₐ) _{100 - x - y - z - b}AₓM' _{y}M"_{z}X_{b} (en % atomique),
dans laquelle M est au moins un élément choisi dans le groupe constitué par Co et Ni, A est au moins un élément choisi dans le groupe constitué par Cu et Au, M' est au moins un élément choisi dans le groupe constitué par Ti, V, Zr, Nb, Mo, Hf, Ta et W, M" est au moins un élément choisi dans le groupe constitué par Cr, Mn, Al, Sn, Zn, Ag, In, les éléments du groupe du platine, Mg, Ca, Sr, Y, les éléments des terres rares, N, O et S, X est au moins un élément choisi dans le groupe constitué par B, Si, C, Ge, Ga et P, a, x, y, z et b satisfont à 0 ≤ a ≤ 0,5, 0 ≤ x ≤ 10, 0,1 ≤ y ≤ 20, 0 ≤ z ≤ 20 et 2 ≤ b ≤ 30, et ledit revêtement isolant ayant une épaisseur moyenne de 2 µm ou moins et consistant en au moins un matériau isolant choisi dans le groupe constitué par les silicates d'aluminium, le silicate de lithium et l'oxyde de magnésium.

2. Alliage nanocristallin selon la revendication 1, dans lequel l'épaisseur moyenne dudit revêtement isolant est de 0,2 µm ou moins.

3. Noyau magnétique fabriqué en laminant ou en enroulant ledit alliage nanocristallin selon la revendication 1 ou 2.

4. Noyau magnétique selon la revendication 3, qui est imprégné avec une résine de type époxy.

5. Procédé pour former un revêtement isolant sur un alliage nanocristallin, qui comprend :
le refroidissement rapide d'un alliage fondu ayant une composition chimique représentée par la formule suivante :
(Fe₁₋ₐMₐ)_{100 - x - y - z - b}AₓM'_{y}M"_{z}X_{b} (en % atomique),
dans laquelle M est au moins un élément choisi dans le groupe constitué par Co et Ni, A est au moins un élément choisi dans le groupe constitué par Cu et Au, M' est au moins un élément choisi dans le groupe constitué par Ti, V, Zr, Nb, Mo, Hf, Ta et W, M" est au moins un élément choisi dans le groupe constitué par Cr, Mn, Al, Sn, Zn, Ag, In, les éléments du groupe du platine, Mg, Ca, Sr, Y, les éléments des terres rares, N, O et S, X est au moins un élément choisi dans le groupe constitué par B, Si, C, Ge, Ga et P, et a, x, y, z et b satisfont à 0 ≤ a ≤ 0,5, 0 ≤ x ≤ 10, 0,1 ≤ y ≤ 20, 0 ≤ z ≤ 20 et 2 ≤ b ≤ 30, pour produire un alliage amorphe ;
le revêtement, sur au moins une surface dudit alliage amorphe, d'une solution contenant au moins un matériau isolant choisi dans le groupe constitué par les silicates d'aluminium, le silicate de lithium et le méthylate de magnésium ;
le séchage de l'alliage amorphe revêtu de solution à une température entre 80 °C et 350 °C ; et
le traitement thermique de l'alliage amorphe séché à une température non inférieure à la température de cristallisation dudit alliage amorphe de façon à former un grain cristallin fin ayant une taille de grain de 30 nm ou moins dans la structure de l'alliage, tout en formant ledit revêtement isolant ayant une épaisseur de 2 µm ou moins et consistant en au moins un matériau isolant choisi dans le groupe constitué par les silicates d'aluminium, le silicate de lithium et l'oxyde de magnésium.

6. Procédé selon la revendication 5, dans lequel ladite solution est appliquée sur ledit alliage amorphe en faisant passer ledit alliage amorphe à travers ladite solution.

7. Procédé selon la revendication 5, dans lequel ladite solution est appliquée sur ledit alliage amorphe en faisant passer ledit alliage amorphe à travers un applicateur à rouleau.

8. Procédé selon la revendication 5, dans lequel ladite solution est appliquée sur ledit alliage amorphe en pulvérisant ladite solution sur la surface dudit alliage amorphe.

9. Procédé selon l'une quelconque des revendications 5 à 8, dans lequel ledit alliage amorphe est revêtu avec ladite solution après avoir soumis la surface dudit alliage amorphe à un traitement d'anodisation.

10. Procédé selon l'une quelconque des revendications 5 à 9, dans lequel ledit alliage amorphe revêtu avec ladite solution est séché en soufflant un air chaud, du gaz argon, du gaz azote ou du gaz hélium sur la surface dudit alliage amorphe.

## Patentansprüche

1. Nanokristalline Legierung mit einer auf mindestens einer Oberfläche vorhandenen Isolierbeschichtung, wobei die nanokristalline Legierung eine durch die nachstehende Formel angegebene chemische Zusammensetzung aufweist:
(Fe₁₋ₐMₐ)_{100-x-y-z-b}AₓM'_{y}M"_{z}X_{b} (in Atom-%),
wobei M mindestens eines der Elemente Co und Ni ist; A mindestens eines der Elemente Cu und Au; M' mindestens eines der Elemente Ti, V, Zr, Nb, Mo, Hf, Ta und W; M" mindestens eines der Elemente Cr, Mn, Al, Sn, Zn, Ag, In, der Elemente der Platingruppe, Mg, Ca, Sr, Y, der Seltenerdelemente, Nb, O und S; X mindestens eines der Elemente B, Si, C, Ge, Ga und P; a, x, y, z und b die Ungleichungen 0 ≤ a ≤ 0,5, 0 ≤ x ≤ 10, 0,1 ≤ y ≤ 20, 0 ≤ z ≤ 20 und 2 ≤ b ≤ 30 erfüllen; und die Isolierbeschichtung eine mittlere Dicke von 2 µm oder weniger aufweist und aus mindestens einem der Isoliermaterialien Aluminiumsilikat, Lithiumsilikat und Magnesiumoxid besteht.

2. Nanokristalline Legierung nach Anspruch 1, wobei die mittlere Dicke der Isolierbeschichtung 0,2 µm oder weniger beträgt.

3. Durch Laminieren oder Wickeln der nanokristalline Legierung nach Anspruch 1 oder 2 hergestellter Magnetkern.

4. Magnetkern nach Anspruch 3, der mit einem Harz des Epoxytyps imprägniert ist.

5. Verfahren zum Herstellen einer Isolierbeschichtung auf einer nanokristalline Legierung, wobei
eine geschmolzene Legierung mit einer durch die folgende Formel angegebenen chemischen Zusammensetzung:
(Fe₁₋ₐMₐ)_{100-x-y-z-b}AₓM'_{y}M"_{z}X_{b} (in Atom-%)
rasch abgeschreckt wird, wobei zur Bildung der amorphen Legierung M mindestens eines der Elemente Co und Ni ist; A mindestens eines der Elemente Cu und Au; M' mindestens eines der Elemente Ti, V, Zr, Nb, Mo, Hf, Ta und W; M" mindestens eines der Elemente Cr, Mn, Al, Sn, Zn, Ag, In, der Elemente der Platingruppe, Mg, Ca, Sr, Y, der Seltenerdelemente, Nb, O und S; X mindestens eines der Elemente B, Si, C, Ge, Ga und P; und a, x, y, z und b die Ungleichungen 0 ≤ a ≤ 0,5, 0 ≤ x ≤ 10, 0,1 ≤ y ≤ 20, 0 ≤ z ≤ 20 und 2 ≤ b ≤ 30 erfüllen,
auf mindestens eine Oberfläche der amorphen Legierung eine Lösung aufgetragen wird, die mindestens eines der Isoliermaterialien Aluminiumsilikat, Lithiumsilikat und Magnesiummethylat enthält,
die mit der Lösung beschichtete amorphe Legierung bei einer Temperatur zwischen 80 und 350 °C getrocknet wird, und
die getrocknete amorphe Legierung bei einer Temperatur wärmebehandelt wird, die nicht unter der Kristallisationstemperatur der amorphen Legierung liegt, um ein feines Kristallkorn mit einer Korngröße von 30 nm oder weniger in einer Legierungsstruktur auszubilden, während gleichzeitig die isolierende Beschichtung in einer Dicke von 2 µm oder weniger ausgebildet wird, die aus mindestens einem der Isoliermaterialien Aluminiumsilikat, Lithiumsilikat und Magnesiumoxid besteht.

6. Verfahren nach Anspruch 5, wobei die Lösung dadurch auf die amorphe Legierung aufgetragen wird, daß die Legierung durch die Lösung geführt wird.

7. Verfahren nach Anspruch 5, wobei die Lösung dadurch auf die amorphe Legierung aufgetragen wird, daß die Legierung durch eine Walzen-Auftrageinrichtung geführt wird.

8. Verfahren nach Anspruch 5, wobei die Lösung durch Aufsprühen auf die Oberfläche der amorphen Legierung aufgetragen wird.

9. Verfahren nach einem der Ansprüche 5 bis 8, wobei die amorphe Legierung nach Anodisieren ihrer Oberfläche mit der Lösung beschichtet wird.

10. Verfahren nach einem der Ansprüche 5 bis 9, wobei die mit der Lösung beschichtete amorphe Legierung durch Aufblasen von Heißluft oder gasförmigem Argon, Stickstoff oder Helium auf ihre Oberfläche getrocknet wird.
